

# UNITED STATES PATENT OFFICE.

EMIL GUSTAV STARK, OF CHEMNITZ, GERMANY.

## PROCESS OF TREATING BRITTLE VEGETABLE FIBERS.

962,173.

Specification of Letters Patent. Patented June 21, 1910.

No Drawing.

Application filed December 20, 1909. Serial No. 534,197.

To all whom it may concern:

Be it known that I, EMIL GUSTAV STARK, Kommerzienrat, a subject of the King of Saxony, and resident of Chemnitz, Saxony, Germany, have invented a new and useful process of treating brittle vegetable fibers, (fibers of capoke, akone, (vegetable silk,) *Calotropis procera*, and the like,) for making them adapted for dyeing and spinning and for enabling them by a special process to be worked up for yarns and twines.

A number of fibers (such as those of capoke, akone, *Calotropis procera*, and on the whole those of the group of *Asclepias*, and the like) which possess a beautiful brilliancy and are well mostly qualified as vegetable silks, are in the natural state, as well known, too brittle for being adapted for uniformly dyeing and spinning. Now it is known that these fibers may be freed from their brittleness when certain so to speak, incrusting, substances (essentially of an organic nature) are taken away from them. This succeeds in treating the fibers by some organic dissolvents such as, for instance, ether, acetone, carbonic disulfid, benzin, benzol, and homologous means. The dissolved substances, and also the dissolvent, may be regained at the same time. The above mentioned substances may also be extracted by means of weak alkaline solutions of Turkey-red, or also by soapy liquors at a heating of 60 to nearly 100 centigrades, suds, tannins, (according to the nature of the fibers).

The last mentioned solutions may be re-

gained and used repeatedly. The extracted fiber is then washed out with water and dried at a moderate temperature, and is in the dried state adapted for uniformly dyeing and spinning, and it may then be worked up to yarns and twines by a special process on machines especially adapted therefor.

Having now described my invention what I claim is:—

1. A process of treating brittle vegetable fibers, such as those of capoke, akone, *Calotropis procera*, and the like, for dyeing and spinning, consisting in treating the fibers with organic dissolvents, washing with water, and drying at a moderate temperature, for working up the fibers to yarns and twines by a special process on machines especially adapted therefor.

2. A process of treating brittle vegetable fibers as mentioned, consisting in extracting the incrusting substances of the fibers by a weak alkaline solution of Turkey-red, or soapy liquors, or suds, or tannins, at a respective degree of heating, washing with water, and drying at a moderate temperature, for working up the fibers thus treated to yarns and twines by a special process on machines especially adapted therefor.

In witness whereof I have hereunto set my hand in the presence of witnesses.

EMIL GUSTAV STARK.

Witnesses:

WILLIAM J. KAUJETSNY,  
WM. WASHINGTON BRUNSWICK,  
JOHANNES BENNDORF.